

(Model.)

A. RUTH.

TOBACCO PIPE AND THE ART OF MANUFACTURING THE SAME.

No. 372,769.

Patented Nov. 8, 1887.

FIG. 1.



FIG. 2.



FIG. 3.



Witnesses

G. G. Somes Jr.  
H. B. Seward

Inventor  
August Ruth  
By E. Edwards Attorney

# UNITED STATES PATENT OFFICE.

AUGUST RUTH, OF ST. LOUIS, MISSOURI.

## TOBACCO-PIPE AND THE ART OF MANUFACTURING THE SAME.

SPECIFICATION forming part of Letters Patent No. 372,769, dated November 8, 1887

Application filed June 18, 1887. Serial No. 241,767. (Model.)

*To all whom it may concern:*

Be it known that I, AUGUST RUTH, of St. Louis, in the State of Missouri, have invented certain new and useful Improvements in Tobacco-Pipes and the Art of Manufacturing the Same; and I do hereby declare the following to be a full, clear, and exact description of the invention, such as will enable others skilled in the art to which it appertains to make and use 10 the same.

My invention relates to an improvement in tobacco-pipes and in the art of manufacturing the same.

Hitherto in the manufacture of corn-cob 15 pipes great difficulty has been experienced in procuring a supply of cobs of suitable diameter to meet the demands, and the consequence has been that the first cost of corn-cob pipes has been much greater than the known abundance of corn-cobs would seem to warrant. Attempts have been made to utilize the smaller cobs by filling the interstices formed by the removal of the kernels with cement and with 20 a glutinous or resinous compound formed by 25 a mixture of corn-starch and gamboge and subsequently dipping the filled cob into a silicate solution. The result has been that while the smaller cobs have been rendered capable of use the nicotine, combined with more or less 30 saliva, has penetrated between the walls of the interstices and the cement or glutinous compound with which they have been filled, and has not only produced discoloration, but has caused the pipe to crack, and has after a short 35 time rendered it worthless.

The object of my present invention is to provide a corn-cob pipe which shall be essentially impervious to nicotine, and which will not discolor by the burning of the tobacco in it.

40 A further object is to provide a pipe of merchantable size from a corn-cob of lesser diameter than has hitherto been deemed suitable for the purpose, and which shall have walls of the desired thickness and strength.

45 A further object is to provide an attractive and durable pipe which may be furnished at a low initial cost.

With these ends in view my invention consists in first treating a corn-cob to render it 50 pliable, and subsequently compressing it to form the bowl of a pipe.

My invention further consists in a corn-cob pipe formed by compressing a corn-cob into the desired shape.

My invention further consists in certain 55 steps of procedure and combinations of elements, as will be hereinafter described, and pointed out in the claims.

In the accompanying drawings, Figure 1 is a sectional view of a mold for compressing the 60 cob, showing the cob or section of the cob in position to be compressed. Fig. 2 is a similar view showing the cob compressed, and Fig. 3 is a view of the completed pipe-bowl.

In its natural state, as may be well known, 65 a corn-cob consists of a central pithy substance around which the thin walls or blades which separate the inner ends of the kernels converge to form a hard wall from one-eighth to one-quarter of an inch in thickness. Such wall is 70 not, however, of uniform thickness in the same cob, and is in many instances soft in places and has small openings where the inner end or point of the kernel extends almost to the pith.

The gist of my invention consists in materially thickening and hardening the above-referred-to wall by compression and rendering it of uniform consistency, and thereby 75 making the use of smaller and imperfect cobs eminently practicable. To accomplish this I 80 first subject the cob to the following treatment, which I find at present to be satisfactory, although I may find it expedient to vary the treatment somewhat, as experience may dictate. The cob or section of cob A, considerably 85 longer than the completed bowl is intended to be, is bored out to a depth such as to leave the cob the desired thickness at the bottom to form the bottom of the pipe-bowl, and the outside is preferably, but not necessarily, 90 trimmed, to give it a more uniform exterior surface. The cob or section of cob A, is then placed in water in which borax is dissolved, and boiled slowly for several hours. The proportion of borax to water should be about one 95 and one-half ounces of borax to one gallon of water for soft cobs and about one ounce of borax to one gallon of water for harder cobs. The harder cobs will also require boiling a longer time than the softer. For example, the 100 softer cobs should be boiled three or four hours and the harder cobs four, five, or six

hours. This has the effect of thoroughly saturating the cob substance with the borax-water and causes the cob to swell in length and thickness and to become elastic. The 5 saturated cob is then taken from the boiling solution and allowed to stand an hour, more or less, and while yet warm is dipped in a thin solution of silicate of soda. It may be either wholly immersed in the solution or may 10 be simply dipped, so as to bring the outer surface into contact with the solution. The latter I find produces satisfactory results. In either case, however, the silicate of soda permeates the swollen pores of the blank and becomes 15 thoroughly incorporated with the cob substance. Before the cob has an opportunity to dry or harden it is placed in a mold, B, shaped to give it the desired form for the completed bowl—in the present instance tapered. 20 It is necessary that the blank should fit the mold without any considerable amount of side play. A block, C, of the suitable thickness, is inserted in the bottom of the mold to form a rest for the lower end of the cob. The block 25 C is interchangeable with a block having a greater or less thickness or a greater or less diameter, to occupy positions at greater or less distances from the bottom of the mold to accommodate cobs of different lengths. A fol- 30 lower or movable platen, D, is provided with a central depending projection, d, adapted to conform to the bore in the cob, and said projection d should be made to extend just to the bottom of the bore when pressed home. The 35 follower is also made interchangeable with others of different depths, to suit different lengths of cobs, and at the same time form pipe-bowls of the same length. Shoulders E at the upper end of the follower serve to limit 40 its movement toward the bottom of the mold, and hence the length of the pipe-bowl.

When the parts have been placed in position, as shown in Fig. 1, the mold is placed in a suitable press of any well-known con- 45 struction, and the follower is forced home into the position shown in Fig. 2. It is locked in this position, preferably by means of hooks e, pivoted to its head, one on each side, which are constructed to engage lugs or studs F on 50 the sides of the mold. When locked, the mold is set aside for the compressed cob or bowl to dry. The drying process may be hastened by the application of heat. A slow heat gives the best results, and the bowl will be in con- 55 dition to be removed from the mold in the course of ten or twelve hours, or sooner if a higher degree of heat be applied. The bowl is then removed from the mold, turned or sand-papered, or both, to give it the desired 60 finish, and a hole formed for the stem.

The pipe-bowl as thus formed has a thick

hard wall of uniform consistency throughout and capable of receiving a high polish.

The molds represented in the accompanying drawings are one of several forms which 65 might be employed to carry out my invention, and hence I do not wish to be understood as confining myself to their particular construction in carrying my method into effect. 70

Having thus fully described my invention, what I claim as new, and desire to secure by Letters Patent, is—

1. The improvement in the art of manufacturing corn-cob pipes, consisting in first 75 treating the cob to render it pliable and subsequently compressing it to form the pipe-bowl.

2. The improvement in the art of manufacturing corn-cob pipes, consisting in first 80 treating the cob to render it pliable and subsequently subjecting it to pressure within a suitable mold to form a pipe-bowl.

3. The improvement in the art of manufacturing corn cob pipes, consisting in first 85 saturating the cob with a solution of borax to render it pliable and subsequently compressing it to form a pipe-bowl.

4. The improvement in the art of manufacturing corn-cob pipes, consisting in first 90 saturating the cob with a solution of borax, then treating it with a silicate solution, and subsequently compressing it to form a pipe-bowl.

5. The improvement in the art of manufacturing corn-cob pipes, consisting in first 95 saturating the cob with a solution of borax, then treating the saturated cob with silicate of soda, and subsequently compressing the cob in a suitable mold to form a pipe-bowl. 100

6. The improvement in the art of manufacturing corn-cob pipes, consisting in the following successive steps: boring the cob to a greater depth than the interior of the finished bowl is intended to be, treating the bored cob 105 to render it pliable, and compressing it in a suitable mold.

7. As an article of manufacture, a compressed corn-cob pipe bowl, substantially as set forth. 110

8. As an article of manufacture, a corn-cob pipe bowl, the walls of which are impregnated with borax and a silicate, and solidified by compression, substantially as set forth.

In testimony whereof I have signed this 115 specification in the presence of two subscribing witnesses.

AUGUST RUTH.

Witnesses:

E. C. SEWARD,  
L. A. CONNER, Jr.